

# United States Patent

[11] 3,625,907

[72] Inventors **Myer Rosenfeld**  
Baltimore;  
**Troy R. Nichols, Bel Air, both of Md.**  
[21] Appl. No. **881,266**  
[22] Filed **Dec. 1, 1969**  
[45] Patented **Dec. 7, 1971**  
[73] Assignee **The United States of America as  
represented by the Secretary of the Army**

[54] **CORROSION INHIBITED PAINT REMOVING  
COMPOSITION**  
8 Claims, No Drawings  
[52] U.S. Cl. .... **252/138,**  
23/53, 117/130, 134/38, 148/6.27, 252/135,  
252/156, 252/387, 252/389, 252/DIG. 8  
[51] Int. Cl. .... **C09d 9/04,**  
C23f 11/18  
[50] Field of Search. .... **252/135,**  
137, 156, 158, 387, 389; 23/53; 204/54 L;  
117/130; 148/6.27; 134/38  
[56] **References Cited**  
UNITED STATES PATENTS  
3,216,945 11/1965 Mankowich..... 252/111

3,034,210 5/1962 **De Long..... 252/389 X**  
2,947,639 8/1960 **Balden..... 117/130 X**  
2,898,246 8/1959 **Hannah..... 252/156 X**  
2,822,325 2/1958 **Tinnon et al..... 204/54 L X**  
1,939,421 12/1933 **Tosterud..... 148/6.27 X**

## OTHER REFERENCES

"Protective Coatings for Metals," by R. M. Burns & W. W. Bradley, 2nd Ed., 1955, pages 156 & 165. The Chemical Formular, Vol. XIII, by H. Bennett, 1967, Page 195.

Primary Examiner—Leon D. Rosdol

Assistant Examiner—Dennis L. Albrecht

Attorneys—Harry M. Saragovitz, Edward J. Kelly and Herbert Berl

**ABSTRACT:** A paint-removing formulation comprising a mixture of: sodium metasilicate pentahydrate, trisodium phosphate dodecahydrate, monosodium phosphate monohydrate, dodecylbenzene sodium sulfonate in conjunction with a small amount of an inhibitor consisting of sodium stannate tetrahydrate or potassium stannate tetrahydrate. In the alternative, the anhydrous forms of the above components may be utilized.

## CORROSION INHIBITED PAINT REMOVING COMPOSITION

The invention described herein may be manufactured, used, and licensed by or for the Government for governmental purposes without the payment to us of any royalty thereon.

This invention relates to a composition having utility in the removal of paints from metals. More particularly, it relates to the inclusion of a small amount of sodium or potassium stannate in a metal paint-removing composition to inhibit the corrosion of aluminum or alloys thereof.

Sodium or potassium chromates are usually utilized in paint removing formulations to inhibit the corrosion of the metal. However, the disposal of waste chromates constitutes a problem in that soluble chromates are poisonous. Accordingly, many municipalities severely limit the chromium concentration permitted to enter effluent streams or waterways. The allowable hexavalent chromium concentrate suggested by the U.S. Public Health Service for the protection of fish is 0.50 milligrams per liter for industrial waste effluent after mixing with receiving water. Therefore, it is often necessary to dilute the waste containing chromate to a permissible level prior to discharging into effluent streams or waterways. When appreciable concentrations of chromates are needed for corrosion inhibition, this becomes a lengthy operation.

formulations set forth in table I below for a period of 1 hour. The panels were then removed from the test solution, rinsed under flowing tap water, dipped into absolute ethyl alcohol and dried with paper toweling. To remove any residual film that had formed during the test, the panels were immersed in concentrated nitric acid at room temperature for 2 minutes. The panels were then rinsed thoroughly under flowing tap water, dipped into absolute ethyl alcohol, dried with paper toweling, and weighed to 0.0001 grams. The difference in weight of the panel after treatment represents loss due to corrosion. It was found that the average weight loss due to the treatment of the panels with nitric acid after immersion of the panels in the cleaning formulation was around 0.05 mg.

The paint removing composition evaluated in this invention consisted of an alkali-type formulation for hot application composed of: sodium metasilicate pentahydrate, trisodium phosphate dodecahydrate, monosodium phosphate monohydrate and dodecylbenzene sodium sulfonate. A corrosion inhibitor consisting of sodium stannate tetrahydrate, potassium stannate tetrahydrate or potassium chromate was utilized. Illustrative examples of the present formulation are set forth in table I below. The ingredients in said table I are calculated on the basis of their hydrated and anhydrous forms.

The utilization of an alkali cleaner without the inclusion of any corrosion inhibitor therein (formulation 1) resulted in an

TABLE I

| Formulation                                                | 1      | 2     | 3     | 4     | 5     | 6     | 7     | 8     | 9     | 10    |
|------------------------------------------------------------|--------|-------|-------|-------|-------|-------|-------|-------|-------|-------|
| Composition (percent by weight):                           |        |       |       |       |       |       |       |       |       |       |
| Sodium metasilicate, pentahydrate                          | 35.08  | 35.07 | 35.04 | 35.07 | 34.31 | 31.69 | 31.69 | 35.07 | 35.07 | 35.01 |
| Trisodium phosphate, dodecahydrate                         | 47.88  | 47.87 | 47.83 | 47.87 | 46.84 | 47.36 | 47.36 | 47.87 | 47.87 | 47.79 |
| Monosodium phosphate, monohydrate                          | 12.03  | 12.02 | 12.01 | 12.02 | 11.77 | 11.89 | 11.89 | 12.02 | 12.02 | 12.00 |
| Dodecylbenzene sodium sulfonate, 86% active                | 5.01   | 5.01  | 5.01  | 5.01  | 4.90  | 4.96  | 4.96  | 5.01  | 5.01  | 5.00  |
| Sodium stannate tetrahydrate                               | 0.03   | 0.11  | 0.02  | 2.18  | 1.10  |       |       | 1.10  | 0.03  |       |
| Potassium chromate                                         |        |       |       |       |       |       |       |       | 0.03  | 0.20  |
| Paint remover, g./100 ml. aqueous solution:                |        |       |       |       |       |       |       |       |       |       |
| Sodium metasilicate, pentahydrate                          | 3.15   | 3.15  | 3.15  | 3.15  | 3.15  | 3.15  | 3.15  | 3.15  | 3.15  | 3.15  |
| Trisodium phosphate, dodecahydrate                         | 4.30   | 4.30  | 4.30  | 4.30  | 4.30  | 4.30  | 4.30  | 4.30  | 4.30  | 4.30  |
| Monosodium phosphate, monohydrate                          | 1.08   | 1.08  | 1.08  | 1.08  | 1.08  | 1.08  | 1.08  | 1.08  | 1.08  | 1.08  |
| Dodecylbenzene sodium sulfonate, 86% active                | 0.45   | 0.45  | 0.45  | 0.45  | 0.45  | 0.45  | 0.45  | 0.45  | 0.45  | 0.45  |
| Sodium stannate                                            | 0.0030 | 0.010 | 0.002 | 0.20  | 0.10  |       |       | 0.10  | 0.003 |       |
| Potassium stannate                                         |        |       |       |       |       |       |       |       | 0.003 | 0.018 |
| Potassium chromate                                         |        |       |       |       |       |       |       |       |       |       |
| Composition (percent by weight as anhydrous):              |        |       |       |       |       |       |       |       |       |       |
| Sodium metasilicate                                        | 36.30  | 36.29 | 36.24 | 36.29 | 35.24 | 35.75 | 35.74 | 36.29 | 36.23 | 36.17 |
| Trisodium phosphate                                        | 37.14  | 37.13 | 37.09 | 37.14 | 36.05 | 36.60 | 36.58 | 37.13 | 37.13 | 37.02 |
| Monosodium phosphate                                       | 18.81  | 18.79 | 18.77 | 18.79 | 18.26 | 18.52 | 18.51 | 18.79 | 18.79 | 18.73 |
| Dodecylbenzene sodium sulfonate, 100% active               | 7.75   | 7.75  | 7.75  | 7.75  | 7.52  | 7.65  | 7.65  | 7.75  | 7.75  | 7.72  |
| Sodium stannate                                            | 0.04   | 0.15  | 0.027 | 2.98  | 1.48  |       |       | 1.52  | 0.04  |       |
| Potassium stannate                                         |        |       |       |       |       |       |       |       | 0.05  | 0.36  |
| Potassium chromate                                         |        |       |       |       |       |       |       |       |       |       |
| Paint remover, g./100 ml. aqueous solution (as anhydrous): |        |       |       |       |       |       |       |       |       |       |
| Sodium metasilicate                                        | 1.81   | 1.81  | 1.81  | 1.81  | 1.81  | 1.81  | 1.81  | 1.81  | 1.81  | 1.81  |
| Trisodium phosphate                                        | 1.85   | 1.85  | 1.85  | 1.85  | 1.85  | 1.85  | 1.85  | 1.85  | 1.85  | 1.85  |
| Monosodium phosphate                                       | 0.94   | 0.94  | 0.94  | 0.94  | 0.94  | 0.94  | 0.94  | 0.94  | 0.94  | 0.94  |
| Dodecylbenzene sodium sulfonate, 100% active               | 0.39   | 0.39  | 0.39  | 0.39  | 0.39  | 0.39  | 0.39  | 0.39  | 0.39  | 0.39  |
| Sodium stannate                                            | .00215 | .0075 | .0015 | 0.15  | 0.075 |       |       | .0773 | .0023 |       |
| Potassium stannate                                         |        |       |       |       |       |       |       |       | .003  | .018  |
| Potassium chromate                                         |        |       |       |       |       |       |       |       |       |       |
| Corrosion (aluminum 2S), average weight loss, mg.          | .35    | 0     | 0     | 0.27  | 0.26  | 0.05  | 0.05  | 0.05  | 0.33  | 0.03  |

It is an object of this invention to provide and disclose a paint-removing composition including a metal-corrosion inhibitor.

It is a further object of this invention to provide and disclose a corrosion inhibitor which is nontoxic to wildlife when discharged in effluent streams and waterways.

Other objects and a fuller understanding of the invention may be had by referring to the following description and claims.

The ability of the present sodium or potassium stannate containing paint removing formulation to inhibit corrosion was evaluated by subjecting metal test panels to the action thereof. Four panels were utilized in the evaluation of each formulation and an average result calculated therefrom. The test panels utilized, which have dimensions of three-fourths inch by 3 inches and a thickness of approximately 0.030 inch, were cut from 2S aluminum (aluminum alloy SAE-AA1100). The panels were cleaned by lightly polishing with No. 150 Alundum paper, washed with acetone, wiped with paper toweling, dipped into absolute ethyl alcohol and again wiped with paper toweling. After being weighed to 0.0001 grams, the test panels were immersed in a boiling aqueous solution of the

average weight loss of 0.35 mg. Negligible corrosion is obtained utilizing 0.03 percent sodium and potassium stannate tetrahydrate as shown in formulation 2 and 8. Formulation 5 indicates that high concentrations, i.e., 2.18 percent by weight of sodium stannate tetrahydrate does not provide sufficient corrosion inhibition. Formulation 4 illustrates that 0.02 percent by weight of sodium stannate tetrahydrate is not adequate to inhibit corrosion. Formulation 10 discloses that 0.20 percent by weight of potassium chromate is essential in order to provide proper corrosion inhibition. This compares with .03 percent by weight of sodium or potassium stannate tetrahydrate.

Although we have described our invention with a certain degree of particularity, we wish it to be understood that we do not desire to be limited to the exact details of formulations shown and described, for obvious modification will occur to a person skilled in the art.

Having described our invention, we claim:

1. A paint stripping composition consisting essentially of about: 34.69-35.07 percent sodium metasilicate pentahydrate; 47.36-48.87 percent trisodium phosphate dodecahydrate;

11.89-12.02 percent monosodium phosphate monohydrate; 46.96-5.01 percent dodecylbenzene sulfonate and a corrosion inhibitor in an amount of about 0.03-1.10 percent selected from the group consisting of potassium and sodium stannate, all amounts being on a weight basis.

2. An aqueous solution of the composition of claim 1 consisting of about 8.98 to 9.08 grams of composition per 100 ml. of solution.

3. An aqueous solution in accordance with claim 1 wherein the corrosion inhibitor is sodium stannate tetrahydrate in an amount of 0.003 to 0.10 grams per 100 ml. of solution.

4. An aqueous solution in accordance with claim 1 wherein the corrosion inhibitor is potassium stannate tetrahydrate in an amount of 0.003 to 0.10 grams per 100 ml. of solution.

5. A paint stripping composition consisting essentially of about: 35.75-36.29 percent sodium metasilicate; 36.60-37.09 per-

cent trisodium phosphate; 18.52-18.79 percent monosodium phosphate; 7.65-7.75 percent dodecylbenzene sodium sulfonate, and a corrosion inhibitor in an amount of about 0.04-1.52 percent selected from the group consisting of potassium and sodium stannate, all amounts being on a weight basis.

6. An aqueous solution of the composition of claim 5 consisting of 5.19-5.30 grams of composition per 100 ml. of solution.

7. An aqueous solution in accordance with claim 5 wherein the corrosion inhibitor is sodium stannate in an amount of 0.002-0.075 grams per 100 ml. of solution.

8. An aqueous solution in accordance with claim 5 wherein the corrosion inhibitor is potassium stannate in an amount of 0.002-0.077 grams per 100 ml. of solution.

\* \* \* \* \*

20

25

30

35

40

45

50

55

60

65

70

75